

[54] **COMPOSITE ARTICLE**[75] Inventor: **Thomas E. Webb**, Richmond, Va.[73] Assignee: **Reynolds Metals Company**,  
Richmond, Va.[22] Filed: **Dec. 18, 1972**[21] Appl. No.: **316,177****Related U.S. Application Data**[63] Continuation of Ser. No. 78,276, Oct. 5, 1970,  
abandoned.[52] **U.S. Cl.** ..... 29/197.5[51] **Int. Cl.** ..... B32b 15/00[58] **Field of Search** ..... 29/197.5[56] **References Cited****UNITED STATES PATENTS**

1,805,448 5/1931 Frary ..... 29/197.5

1,865,089 6/1932 Dix ..... 29/197.5

|           |         |               |          |
|-----------|---------|---------------|----------|
| 1,975,105 | 10/1934 | Keller .....  | 29/197.5 |
| 2,122,535 | 7/1938  | Nock .....    | 29/197.5 |
| 3,400,450 | 9/1968  | Nock .....    | 29/197.5 |
| 3,482,951 | 12/1969 | Hubbell ..... | 29/197.5 |

**OTHER PUBLICATIONS***"Metals Handbook", Vol. 1, 8th Edition, Published  
1961, American Society for Metals, p. 917.**Primary Examiner—Hyland Bizot**Attorney, Agent, or Firm—Glenn, Palmer, Lyne &  
Gibbs*[57] **ABSTRACT**

An alclad sheet product, suitable for porcelain enameling, having an aluminous metal cladding layer of 3003 alloy, for example, and an adjoining layer of an aluminum base alloy containing about 2 to 3 percent copper, up to about 0.4 percent manganese, and about 0.2 to 0.6 percent magnesium.

**7 Claims, No Drawings**

## COMPOSITE ARTICLE

This application is a continuation of Ser. No. 78,276 filed on Oct. 5, 1970, now abandoned.

The present invention relates to a composite aluminum metal article, typically in sheet form, having an outer cladding layer suitable for porcelain enameling and an adjoining core layer which is susceptible to strengthening under thermal conditions incident to porcelainizing treatment. The composite is adapted for such uses as making coated aluminum utensils, including those having an interior non-stick coating, and the core and cladding layers are selected to provide improved resistance to exfoliation and blistering.

## BACKGROUND OF THE INVENTION

Aluminum utensils are commonly provided with a TFE coating on their interior cooking surfaces. Porcelain enameling is used to finish the exterior surfaces of these and other products made of clad composites. The 20 aluminous materials used for such purposes may be a commercial grade of aluminum (1XXX series) or a high aluminum content alloy such as 3,003, either along or as cladding on a stronger base alloy providing greater rigidity. Two such clad composites previously used are 3,003 clad 7,005-type alloy and 1,100 clad 7,004-type alloy.

In these applications a cladding of 1,100 or 3,003 aluminum has been selected primarily on the basis of its suitability for porcelainizing or TFE coating operations, while the 7,004 and 7,005 type alloys have been chosen for their responsiveness to strengthening under thermal conditions incident to such operations. It has been found that the resulting combinations are less than ideal, however, because these cladding materials are not sufficiently anodic to such core alloys to provide electrolytic protection. Thus, in the event of a scratch or other discontinuity which allows access of corrosive food constituents or water and other substances used for cleaning purposes, a form of corrosion may occur which tends to spread laterally along and through the core layer, resulting in exfoliation and blistering.

An object of the present invention is to provide an alclad composite exhibiting improved resistance against such attack, while still employing conventional cladding materials adapted for porcelain enameling.

## SUMMARY OF THE INVENTION

It has been found that an alclad copper-bearing aluminum base core alloy provides improved results with respect to corrosion resistance of the composite, in that such an alloy serves to limit attack to minor pitting of a localized nature. In accordance with the invention, the cladding layer is bonded to a base layer of an alloy consisting essentially of aluminum, about 2 to 3 percent copper, up to about 0.4 percent manganese, and about 0.2 to 0.6 percent magnesium by weight. This alloy may also contain the usual incidental impurities as well as minor alloying elements in customary amounts for recognized purposes, including, for example, up to about 0.8 percent silicon, 0.7 percent iron, 0.1 percent chromium, 0.25 percent zinc and 0.2 percent titanium.

The cladding may be applied on one or both surfaces of the base layer. A preferred cladding alloy is 3,003, but other conventional aluminous metal cladding materials are suitable, such as aluminum and high aluminum

content alloys capable of affording electrolytic protection, particularly those of the 1XXX and 3XXX series (Aluminum Association designation).

## EXAMPLE

The following example illustrates the practice of the invention and its presently preferred embodiment:

An ingot was prepared having a core composed of a copper-bearing aluminum base alloy and having 3,003 10 alloy cladding (10 percent) on both sides, then rolled to 0.102" gage, blanked into suitable circles, and subjected to thermal treatment to simulate porcelainizing and TFE coating cycles. The core composition (alloy X2,036) in weight percentages was:

15

|           |                   |
|-----------|-------------------|
| 0.50 max. | Si                |
| 0.50 max. | Fe                |
| 2.2-3.0   | Cu                |
| 0.10-0.40 | Mn                |
| 0.30-0.6  | Mg                |
| 0.10 max. | Cr                |
| 0.25 max. | Zn                |
| 0.15 max. | Ti                |
| Others,   | each .05 max.     |
|           | total 0.15 max.   |
|           | Balance aluminum. |

25

For purposes of comparison, reference specimens were prepared from conventional 3,003 clad 7,005-type alloy. Exfoliation tests (5-day MASTMAASTS standard) were performed on annealed materials, and also on those treated for 10 minutes at 1000°F. and fan cooled (to simulate porcelainizing) and for 15 minutes at 750°F. and air cooled (to simulate TFE coating).

30

The conventional materials showed moderate to severe blistering both in annealed and heat treated condition.

35

In contrast, the composite materials of the present invention showed only slight pitting (no blistering or exfoliation attack) in either condition.

40

A clad product of this sort is known commercially as "Type 36 porcelain enameling sheet." Its core alloy X2036 was registered with the U.S. Aluminum Association on Aug. 13, 1970, by the assignee of this application.

45

Alclad X2036 alloy in the form of such porcelain enameling sheet (PE-36) is suitable for conventional fabricating operations incident to making various types of cooking utensils, particularly pans and the like having a TFE non-stick coating or a porcelain enamel coating, or both, and such coatings are readily applied to a cladding surface of the composite sheet. The invention embraces the clad product itself, its use in making cooking utensils, and the method of applying such coatings.

50

The term "Alclad" is used here in the accepted sense to indicate a bonded composite having a layer of aluminum or corrosion-resistant aluminum alloy which is anodic to the core of structurally stronger aluminum alloy it covers, thus physically and electrolytically protecting the core alloy against corrosion.

55

What is claimed is:

60

1. A clad article having a cladding of 1,100 aluminum on a core alloy consisting essentially of aluminum, about 2 to 3 percent copper, about 0.2 to 0.6 percent magnesium and up to about 0.4 percent manganese by weight.

65

2. A clad article having a cladding of 3,003 alloy on a core alloy consisting essentially of aluminum, about 2 to 3 percent copper, about 0.2 to 0.6 percent magne-

sium and up to about 0.4 percent manganese by weight.

3. Type PE36 porcelain enameling sheet comprising an aluminum base alloy core consisting essentially of aluminum, 2.2 to 3.0 percent copper, 0.3 to 0.6 percent magnesium and 0.10 to 0.40 percent manganese by weight; and a cladding of alloy 3,003 that is anodic to said core alloy and effective cooperatively therewith to avoid exfoliation and blistering.

4. A cooking utensil made of sheet according to claim 3.

5. An article comprising a clad composite having a

cladding layer composed of aluminum base alloy 3,003, and an adjoining core layer of an alloy consisting essentially of aluminum, about 2.2 to 3 percent copper, about 0.10 to 0.40 percent manganese and about 0.30 to 0.6 percent magnesium, by weight, with incidental elements and impurities not exceeding 0.8 percent silicon, 0.7 percent iron, 0.1 percent chromium, 0.25 percent zinc and 0.2 percent titanium.

6. The article of claim 5 in the form of sheet.

7. The article of claim 5 in the form of sheet, having said cladding on both sides of the sheet.

\* \* \* \* \*

15

20

25

30

35

40

45

50

55

60

65

UNITED STATES PATENT OFFICE  
CERTIFICATE OF CORRECTION

Patent No. 3,850,585 Dated Nov. 26, 1974  
Inventor(s) Thomas E. Webb

It is certified that error appears in the above-identified patent and that said Letters Patent are hereby corrected as shown below:

In col. 1 at lines 23, 26, 27, 28, 31 and 66; in col. 2 at lines 9, 14 and 27; in line 1 of claim 1, in line 1 of claim 2, in line 5 of claim 3 and in line 2 of claim 5, no comma should be present in any of the four-digit alloy designations. Thus, for "3,003" read --3003-- and for "1,100" read --1100--.

Signed and sealed this 18th day of February 1975.

(SEAL)  
Attest:

RUTH C. MASON  
Attesting Officer

C. MARSHALL DANN  
Commissioner of Patents  
and Trademarks